

Patented Nov. 15, 1927.

1,649,675

# UNITED STATES PATENT OFFICE.

JUSTUS ELLENBERGER, OF WIESBADEN, GERMANY, ASSIGNOR OF ONE-HALF TO BRITISH GLUES AND CHEMICALS LIMITED, OF LONDON, ENGLAND, A COMPANY OF GREAT BRITAIN.

## PROCESS FOR THE MANUFACTURE OF ARTIFICIAL HORN.

No Drawing. Application filed April 12, 1926, Serial No. 101,558, and in Germany January 9, 1925.

This invention relates to artificial horn and the manufacture of the same and has for its object to provide an improved process by which a satisfactory article is produced 5 from cheaper materials than those heretofore employed.

In carrying out the present invention the residue of nitrogenous substances from which the glue-forming matter has been re-10 moved, is used.

In the manufacture of glue and gelatine from chrome leather by boiling it with slightly alkaline water in the presence of a suitable magnesium compound such as caustic burnt magnesite, there is left after the glue or gelatine has been removed a scutch or residue that contains approximately 20% nitrogenous matter (with which is admixed chromium and magnesium compounds) and 20 about 80% water. Similar nitrogenous material derived from animal sources (hereinafter deemed to be included in the term "scutch") may be employed.

According to the present invention the 25 scutch which is of a pulp-like nature is firstly strained through a metal screen to eliminate any foreign matter and may be pressed to reduce the water content. It is then mixed with an absorbent binding material, such as saponified resin, or a suitable 30 hygroscopic substance such as calcium chloride, magnesium chloride or the like. The mixture is afterwards thoroughly kneaded and subjected to pressure. It is then placed 35 in a solution of formaldehyde for a suitable period and afterwards rinsed and dried as is hereinafter more particularly described.

In some cases an organic acid such as 40 acetic acid is added before the material is pressed in order to increase its suppleness and to wholly or partially render soluble any chromium that may be present.

Fillers, such as china clay, lithopone, 45 barytes or similar substances may be incorporated with the mixture before the pressing operation.

A suitable dye may be added to the material undergoing treatment either before or 50 after the pressing process or both before and

According to one mode of carrying out the present invention, when the nitrogenous material used is the scutch derived from degluing chrome leather it is first strained

as hereinbefore stated. Fifteen per centum 55 of resin (such as colophony) calculated on the dried finished product is now mixed by kneading in a machine of known construction after which a sufficient quantity of alkali to saponify the resin is added. 60

The moisture content of the mixture should be about 30% according to the quality of the horn required. This proportion can be effected by pressing the scutch before the kneading operation as hereinbefore de-65 scribed.

A small quantity of acetic acid (varying from 1% to 5%) is now added to produce the desired suppleness of the mixture and to enable the desired proportion of the 70 chromium content to be removed in the subsequent treatment.

The mixture is now removed to a moulding press of known construction in which it is subjected to a pressure of 200 to 600 atmospheres and a temperature gradually rising to 100 degrees Celsius and then gradually falling. 75

When the moulded material is in a suitable condition it is removed to a bath containing a 3% to 6% solution of formaldehyde in which it is allowed to remain until it is completely hardened. It is then removed, rinsed and slowly dried in air at a 80 suitable temperature. 85

By means of the hereinbefore described process an artificial horn is produced.

In some cases calcium chloride or magnesium chloride may be used as a binder 90 instead of saponified resin.

Obviously the degree of removal of the glue and gelatine during the degluing step will depend on several factors and may be more or less complete and the term "degluing" is used in the claim in this sense. 95

I claim:

A process for the manufacture of artificial horn comprising, degluing leather scrap whereby a nitrogenous residue is left, adding resin to said residue, thereafter adding 100 a sufficient quantity of alkali to saponify the resin, molding the mixture and hardening with formaldehyde.

In testimony whereof I have signed my name to this specification at Frankfort on 105 Main, Germany, this thirtieth day of March, 1926.

JUSTUS ELLENBERGER.